

Patented Dec. 18, 1934

1,984,968

# UNITED STATES PATENT OFFICE

1,984,968

## METHOD OF PRODUCING PYROPHOSPHATES

Augustus H. Fiske, Warren, and Charles S. Bryan, East Providence, R. I., assignors to Rumford Chemical Works, Rumford, R. I., a corporation of Rhode Island

No Drawing. Application August 31, 1931,  
Serial No. 560,510

1 Claim. (Cl. 23—107)

This invention relates to the production of pyrophosphates in general and especially to the production of acid sodium pyrophosphate, and particularly to a process for producing the same by which certain economies in the manufacture are perfected and by which a high grade pyrophosphate is produced well adapted for use in baking powders or for like purposes as for leavening and wherever a pyrophosphate of any nature

10 may be required.

Our procedure, as well as the advantages, will be set forth in the following specification in which we will disclose so much of the manufacture as is herein immediately involved and which

15 serves as a basis of the disclosure of our invention.

We employ in our process phosphoric acid free from undesirable impurities such as, lead, copper, arsenic, fluorine, etc., but containing the normal amount of iron and aluminum (up to 2% approximately, calculated on the basis of  $Al_2O_3$  and  $Fe_2O_3$ ). This acid is preferably at about 50° to 55° Baumé or may be at even greater strength. Our usual solution will contain about 70% to 25 75% of orthophosphoric acid and while we do not wish to limit our invention to these exact strengths, it has been our experience that phosphoric acid solutions of about this strength give the best results in processing of the materials.

30 In explaining a characteristic procedure according to our invention we may consider for an example our process as applied to the production of acid sodium pyrophosphate as this material is commercially the most common of the pyrophosphates. We do not wish, however, to limit our invention to the preparation of this pyrophosphate but make reservation that the process as described in this specification by us is applicable to the manufacture of other pyrophosphates both

40 acid and basic and neutral and containing a variety of bases—such as calcium, magnesium, and potassium.

In our process as applied for example to the manufacture of acid sodium pyrophosphate, the phosphoric acid is thoroughly mixed with the calculated amount of powdered or granular sodium hydroxide (caustic soda) in an oven which may be heated to a carefully regulated temperature. During the reaction as it takes place between the acid and the hydroxide, sufficient heat is evolved to evaporate off the greater part of the uncombined moisture and at the same time the heat of the oven which is regulated to almost exactly 200° C. but not to exceed in any event 220° C., drives off the molecule of combined water producing acid sodium pyrophosphate directly from the oven. Thus the material is formed from its ingredients in one operation.

60 This process may be carried out in an oven with a travelling hearth containing ploughs or stir-

ers. Thus the phosphoric acid and sodium hydroxide are introduced in the travelling hearth at one end of the oven and the finished acid sodium pyrophosphate is produced at the other end of the oven in a dry friable condition ready for

5

Our process as will be noted is one of extreme simplicity and in this simplicity lies many of its advantages. In it we have the advantage of highly concentrated phosphoric acid in place of the usual more dilute solutions.

The sodium hydroxide or caustic soda in place of soda ash is of great advantage both in processing and in resultant product. One of our great advantages and characteristic features is that the material can be produced in a dry condition without the usual delay of passing through the process of evaporation and this is particularly important because in many systems it is necessary for commercial production to dry the material in a vacuum drier to prevent the material melting in the oven and discoloring in this stage of the process of manufacture, whereas our material is treated in the oven at about 200° during the process of formation where melting at high temperature is reduced to a minimum and similarly discoloration from this source is minimized.

By our process we produce a pyrophosphate retaining a small amount of iron and aluminum pyrophosphates which are advantageous in baking powder as they have a tendency to slow the reaction of the pyrophosphate with the bicarbonate of soda.

In our process there is no tendency to froth as in processes using more dilute acid and/or sodium carbonate or other carbonates in place of the oxides or hydroxides. This frothing is very hard to control in an oven in such a process and makes difficulties in handling. We do not, therefore, recommend the use of solutions of phosphoric acid much below 50° Baumé, but, nevertheless, we feel that the material even though it be of not such good quality may be made at a lower strength of the acid, although it would require less advantageous handling and mixing and generally necessitate a slowing up of the process and resulting decrease in economy.

What we therefore claim and desire to secure by Letters Patent is:

That method of producing an acid sodium pyrophosphate free from metaphosphate consisting in mixing to reactive dryness, without evaporation, phosphoric acid of substantially 50 to 55° Baumé with caustic soda while heating at atmospheric pressure to substantially 200° C. until a permanent dry acid sodium phosphate is formed.

AUGUSTUS H. FISKE.  
CHARLES S. BRYAN.

60